

## UNITED STATES PATENT OFFICE

2,471,918

## ELECTRODEPOSITION OF COPPER

Karl S. Willson and David G. Ellis, Cleveland, Ohio, assignors to The Harshaw Chemical Company, Cleveland, Ohio, a corporation of Ohio

No Drawing. Application December 12, 1946, Serial No. 715,626

3 Claims. (Cl. 204—52)

1

This invention relates to electrodeposition of copper and more particularly to improved processes and solutions for electrodeposition of bright copper.

We have now discovered that by the inclusion in the copper cyanide plating solution of a suitable quantity of an organic compound of the formula



which is suitably soluble in the solution and stable therein and wherein R represents a radical of the class consisting of alkyl and aryl radicals containing not more than six carbon atoms, we are able to produce an electrodeposit of small grain size and having substantial lustre. That is, when such a deposit is made, it can be built up to substantial thickness, three ten thousandths of an inch and more, and still exhibit greatly improved lustre as compared with the usual cyanide copper bath. Agitation of the solution results in improvement in lustre and makes possible the use of much higher current density, e. g. increase from 10 ASF to 60 ASF. Interruption of the current at intervals, e. g. 1 minute on, 10 seconds off, reversal of the current every few seconds or use of alternating current superimposed on the direct current, all tend to produce improved lustre and more uniform deposits.

Examples of compounds which have the requisite solubility and stability are:



The compound to be suitable should have adequate solubility in the copper cyanide bath to make possible the maintenance in solution of a sufficient quantity of the addition agent to achieve the desired result. The brightening effect or grain size reduction can be achieved in greater or lesser degree with very small amounts of the indicated addition agents. In general the concentration of addition agent should not be less than 0.10 gram per liter and when maximum brightness has been achieved, it is not profitable to increase the concentration further. In general 2.5 grams per liter may be taken as a sufficient concentration. Any of the compounds mentioned having a solubility in the copper cyanide solution of at least 0.10 gram per liter may be expected to achieve

2

the benefits of the invention in substantial degree at a concentration of 0.10 gram per liter and they may be used in quantity up to 3.75 grams per liter.

- 5 An aqueous alkaline plating bath may be employed containing 4 to 20 ounces of CuCN per gallon (30 to 150 grams per liter) and the requisite amount of NaCN. The preferred pH range is 9.5 to 11.5 but good results may be had from 8.5 to 10 12.5. Free cyanide content may be from 0 to 11.5 grams per liter or more. In general, increase of free cyanide is desirable with increasing CuCN content. The temperature is preferably maintained between 130° F. and 150° F. although good results can be had between 120° F. and 160° F.
- 15 Current is passed through the above indicated solutions from a copper anode to a cathode at a cathode current density of from a very low value up to 60 amperes per square foot.
- 20 Preferred solutions and plating conditions would be, for example:

## Example I

|                    |                      |
|--------------------|----------------------|
| CuCN               | 120 grams per liter  |
| Free cyanide       | 3.75 grams per liter |
| 2-acetyl thiophene | 3.75 grams per liter |
| Water              | Remainder            |
| pH                 | 10.5                 |
| Temp.              | 140° F.              |
| Current density    | 40 ASF.              |

## Example II

|                     |                      |
|---------------------|----------------------|
| CuCN                | 120 grams per liter  |
| Free CN             | 4.5 grams per liter  |
| 2-benzoyl thiophene | 3.75 grams per liter |
| Water               | Remainder            |
| pH                  | 10.0                 |
| Temp.               | 140° F.              |
| Current density     | 30 ASF.              |

- 40 Having thus described our invention, what we claim is:

1. In a process for electrodepositing bright copper, the step which comprises electrolyzing an aqueous alkaline copper cyanide solution and a minor proportion of a soluble acyl thiophene compound corresponding to the formula



55 where R represents a radical of the class consisting of alkyl and aryl radicals having not more than six carbon atoms, the copper cyanide concentration being from 30 to 150 grams per liter

and the concentration of the acyl thiophene compound being from 0.10 to 3.75 grams per liter.

2. In a process for electrodepositing bright copper, the step which comprises electrolyzing an aqueous, alkaline copper cyanide solution and a minor proportion from 0.10 to 3.75 grams per liter of acetyl thiophene.

3. In a process for electrodepositing bright copper, the step which comprises electrolyzing an aqueous, alkaline copper cyanide solution and a minor proportion from 0.10 to 3.75 grams per liter of benzoyl thiophene.

KARL S. WILLSON.  
DAVID G. ELLIS.

#### REFERENCES CITED

The following references are of record in the file of this patent:

#### UNITED STATES PATENTS

| Number    | Name            | Date          |
|-----------|-----------------|---------------|
| 2,410,844 | Signaigo et al. | Nov. 12, 1946 |